

## UNITED STATES PATENT OFFICE.

JOHN K. TULLIS, OF NEW YORK, N. Y., ASSIGNOR, BY MESNE ASSIGNMENTS, TO  
GELTAN COMPANY, OF NEW YORK, N. Y., A CORPORATION OF DELAWARE.

## LEATHER MANUFACTURE.

No Drawing.

Application filed March 3, 1923. Serial No. 622,642.

This invention relates to the production of leather of superior quality by introducing gelatine into the leather at the proper time, thereby obtaining leather which is more flexible and pliable and is less apt to crack upon being bent and which will wear better and be less liable to deteriorate with age.

Heretofore it has been thought to be desirable to introduce gelatine from an outside source into the hides in order to improve the qualities of the leather, but attempts to do this satisfactorily have failed largely because of the fact that the gelatine would become coated upon the outside surfaces of the leather without penetrating the interior to the extent desired or to a sufficient degree to give the best results.

By the present invention gelatine may be introduced into the leather by means of a carrier, such as a salt which will act in this capacity, after the ordinary tanning operations have been performed and while the leather is still in the damp condition. The gelatine may be obtained from ordinary sources or it may be obtained from the flesh and other products that are removed from the hides during the dehairing and fleshing operations of the raw hides that are to be treated by the process of this invention. The leather that is to have the gelatine introduced thereto may be chrome tanned leather or it may have been tanned by using the ordinary vegetable tanning extracts such as quebracho, hemlock, chestnut, oak bark, mangrove, spruce, etc., or synthetic tanning materials such as the formaldehyde condensation products, for example. The gelatine and salt will preferably be first intimately mixed with vegetable tanning extracts and a sufficient amount of tallow and cod liver or similar oil to make a paste, and this composition may then be introduced into the tanned leather while the leather is still in a damp condition in an oil wheel or drum. Without intending to restrict myself to the particular proportions or ingredients, I will give the following as a specific example illustrative of the invention:—A mixture may be made consisting of approximately equal parts of gelatine, a salt such as sodium chloride, and a vegetable tanning extract

such as ordinary commercial quebracho. About two parts of this mixture may be compounded with about one part of tallow and cod liver oil, the tallow and oil being of about equal proportions and the whole may be thoroughly mixed to form a paste-like composition. After the hides have been tanned in the usual or well known manner and while they are still in a damp condition they may be treated from about 20 minutes to 1 hour with the paste or composition in a wheel or drum such as is commonly used in this art.

It has been found that when the tanned leather has been treated in the manner above described the gelatine is caused to penetrate the leather instead of merely coating its surface thereby bringing about the result long sought for, and greatly improving the quality of the leather itself.

## I claim:

1. A composition of matter comprising gelatine, a salt and tanning material.
2. A composition of matter comprising gelatine, a salt, tanning material, tallow and oil.
3. A composition of matter comprising gelatine, NaCl and a vegetable tanning extract.
4. A composition of matter comprising substantially equal parts of gelatine, NaCl and a vegetable tanning extract, and about half as much tallow and a non-drying oil.
5. The process which comprises tanning leather and treating it while damp with a composition containing gelatine and a salt.
6. The process which comprises tanning leather and treating it while damp with a composition containing gelatine and sodium chloride.
7. The process which comprises tanning leather and treating it while damp with a composition containing gelatine, a salt, tanning material, tallow and oil.
8. Leather having gelatine distributed therein.
9. Leather having gelatine substantially uniformly distributed therethrough.

In testimony whereof I affix my signature.

JOHN K. TULLIS.